

## UNITED STATES PATENT OFFICE

2,012,966

## ALLOY

Harlan J. McFadgen, Sr., Oakland, Calif., assignor to Chrome Alloys Manufacturing Company, Oakland, Calif., a copartnership composed of Franklin Warner and Harlan J. McFadgen, Sr.

No Drawing. Application May 31, 1932, Serial No. 614,611

## 2 Claims. (Cl. 75—1)

My invention relates to alloys, and has particular reference to alloys formed between metals having a high melting point and metals having a low melting point.

5 Various attempts have been made to produce alloys between metals having a high melting point and other metals having a low melting point, but the percentage of low melting point metals which could be alloyed, has been relatively small, 10 in some instances the low melting point metal suffering considerable loss in introduction into the composition. For example, alloys have been attempted between metals such as nickel and/or chromium, which have high melting points, and 15 copper and zinc having low melting points, with little success in obtaining an alloy which has a high percentage of the zinc or copper, while other attempts to form such alloys have resulted in the precipitation of the nickel or chromium from 20 the molten mass preventing reasonable assurance that the finished product would have the desired percentages of high and low melting point metals.

It is, therefore, an object of this invention to 25 provide an alloy which includes as its constituent elements one or more metals having a high melting point and having a relatively large percentage of low melting point metal, such as zinc.

Another object of the invention is to provide 30 an alloy which has the characteristics of being non-corrosive and non-tarnishing in the presence of salt water, chlorine and the most acid fumes, and which also has the characteristic of being relatively strong and of high tensile strength.

Another object of the invention is to provide 35 an alloy containing a large percentage of zinc which has the characteristic of not only having relatively high tensile strength, but also having a relatively high yielding point.

Another object of the invention is to provide a 40 relatively inexpensive alloy which has the property of a fine-grained structure readily machined and which, when polished, presents the high luster finish of chromium throughout all portions of the structure.

Another object of the invention is to provide a 45 method of producing an alloy between high melting point metal and low melting point metals.

Another object of the invention is to provide a 50 method of introducing a relatively large percentage of low melting point metal, such as zinc, into alloys containing high melting point metals without appreciable loss of the low melting point metals.

Another object of the invention is to provide a flux which may be employed in forming an alloy between high melting point metals and low melting point metals.

In various types of construction, it is desirable to employ a metal which is relatively hard, and which has a high tensile strength, but which, at the same time, includes the properties of receiving and retaining a high polish, presenting a silvery appearance, such as that known in the 10 art as a "chromium finish". Typical constructions of this type are marine hardware, which is to be exposed to the action of salt water, in which the non-corrosive feature is of great importance in retaining the desired finish or polish upon the 15 metal. At the same time, such devices must be able to withstand considerable strains and stresses.

I have discovered that an alloy particularly adapted for this use, may be made in a relatively 20 inexpensive manner from relatively inexpensive ingredients. For example, a metal which contains a large percentage of zinc may be employed with a small percentage of chromium, the combination of these two metals giving the desired 25 non-corrosive properties, and also producing a metal having the "white" color desired for a pleasing appearance.

Also, this combination of zinc and chromium 30 may be rendered very hard and very tough by the introduction of a relatively high percentage of copper, to which may be added other tougheners, such as manganese, iron, tin, nickel, and other metals. However, it will be noted that the finished 35 alloy is formed of large percentages of relatively inexpensive metals, that is, zinc and copper, which constitute approximately 80 to 90% of the finished product, and are both relatively inexpensive metals, while the quantity of more expensive materials, such as nickel and chromium, 40 employed is relatively small constituting not over 14 to 15% of the finished product.

For example, I find that an alloy formed from 45 copper, nickel, zinc, manganese, iron and chromium produces a highly desirable material for substantially all purposes, for which a strong, sturdy, tough metal is to be used to be exposed to water or other corrosive or tarnishing atmospheres, and in which it is desired that the polished luster finish be consistently maintained 50 over a long period of time.

Such a material may be formed from the following constituents in substantially the following proportions:

|                    | Percent  |
|--------------------|----------|
| Copper             | 40 to 50 |
| Zinc               | 40 to 50 |
| Nickel             | 5 to 10  |
| 5 Manganese        | 1 to 2   |
| Chromium           | .1 to .5 |
| Tin                | .5 to 1  |
| Phosphorous copper | .1 to .2 |

Such alloys having approximately the following 10 physical properties:

|                       |                                                   |
|-----------------------|---------------------------------------------------|
| Color                 | White                                             |
| Weight per cubic inch | .325 lb.                                          |
| Tensile strength      | 77,210 lbs. per square in.<br>(standard test bar) |
| Elongation in inches  | 10% of 2 inches                                   |
| Scleroscope           | 32.5 scale reading                                |
| Melting point         | 2,010° F.                                         |
| Yielding point        | 54,634 lbs. per sq. in.                           |
| 20 Reduction in area  | 9.2%                                              |
| Brinell hardness      | 10 m. m. Ball Brinell<br>scale reading            |
| 500 K.G. load         | 153 (scale reading)                               |
| Rockwell              | B-79.1 (Rockwell scale reading)                   |

25 The various ingredients may be combined in the following manner, the amounts indicated forming a quantity of finished alloy of about 180 lbs:

30 A crucible or electric furnace may be used for the melting of the various ingredients, the charge being substantially as follows: On the bottom of the crucible or furnace should be placed 5 pounds of zinc, 10 pounds of copper,  $\frac{1}{4}$  pound of chromium in the form of ferro chromium containing approximately 60% chromium, approximately 1 pound of a flux to be hereinafter described, then a charge of about 25 pounds of copper and nickel, which I prefer to employ in the form of copper-nickel shot containing approximately 50% copper and 50% nickel. Then approximately an additional pound of the flux should be spread on top of the charge, again a layer of approximately 25 pounds of copper-nickel shot, and then approximately 1 pound of the flux should be spread upon the charge.

40 The charge may then be heated to about 3,000° F. which will cause the melting of the material in the crucible.

45 By charging the crucible in the manner set forth, the zinc and copper will be at the bottom of the charge so that as the copper-nickel shot is melted, the nickel constituents will flow downwardly through the flux to meet the molten zinc and copper and mix properly therewith. The flux will melt and form a protective coating upon the top of the molten mass to prevent oxidation of the constituents and of the preliminary alloy of copper, nickel, chromium and zinc so formed.

50 I prefer to employ the nickel in the form of the copper-nickel shot, primarily because the melting point of this combination of metals is considerably below that of nickel alone, thus rendering it unnecessary to bring the crucible up to the temperature at which nickel alone would melt. 55 Moreover, nickel-copper shot when melted will more readily mix with the copper and zinc charge of the crucible than would nickel alone.

60 After the initial charge has been thoroughly melted, I add the manganese copper, stirring the molten mixture repeatedly during the introduction of the manganese copper. I then add 45 pounds of copper in small quantities of approximately 3 to 8 pounds each, letting each small quantity of copper melt thoroughly before add-

ing more. At this time, approximately  $\frac{1}{4}$  pound of the aluminum should be added to act as a deoxidizer and cleanser. The introduction of the copper will tend to lower the heat of the mixture, and it should be reheated to about 2500° F. and then the crucible allowed to cool to about 1800°.

65 The zinc to be added should be warmed and charged, while the molten mass is at about 1800° in small charges of about 10 pounds each, immersing each of the small charges immediately 10 below the flux and slag and stirring the mixture rapidly while holding the charge immersed. The charging should be repeated until approximately 70 pounds of zinc has been charged and melted into the mixture.

15 After the introduction of the zinc, the mixture should be reheated to about 2250°, after which the charge is ready to draw. Immediately prior to the drawing of the charge, the flux should be skinned off and about 2 pounds of tin added and stirred well into the molten mass. At this time also about  $\frac{1}{4}$  pound of aluminum and  $\frac{1}{4}$  pound 20 10% phosphorous copper should be added and stirred well into the mixture, after which the molten mass should again be skinned clean, the 25 temperature of the mass at this time being tested to insure that as the skimmer is drawn across the top of the crucible it leaves a trailing wave of about  $\frac{1}{4}$  inch behind it, this condition obtaining when the mixture is at the most desirable 30 temperature for casting.

35 The above noted ingredients and quantities will produce approximately 180 pounds of the finished product, which may be then cast in any suitable 35 shape in the same manner as brass or similar alloys.

40 It will be noted that only a small quantity of copper and zinc is used in the initial charge and that after the nickel and chromium are melted the remainder of the copper and the zinc is added 40 in such small quantities that there is no opportunity for the mass to be chilled by the introduction of the copper and zinc, nor is there an opportunity for the nickel and chromium to precipitate or amalgamate and set in the crucible.

45 It will also be observed that the introduction of the copper and zinc is made after the initial charge has been melted and it is covered with the flux. Ordinarily, the introduction of zinc into a mass at the temperature indicated herein would 50 cause the zinc to immediately vaporize and be blown out of the mix, thereby losing substantially all of the zinc as it is introduced into the crucible. I prevent this occurrence by employing a flux which is relatively heavy and which, if the zinc is 55 introduced below the flux, by immediately immersing the zinc into the molten mass below the flux, the zinc will be melted and alloyed with the remaining constituents without having an opportunity to oxidize or vaporize.

60 The flux which I prefer to use includes a relatively large percentage of ground glass and borax to which is added a considerable quantity of ground shell. The particular shell employed is preferably one having a low lime content and it 65 is preferably one which is of bone character, rather than of a calcium carbonate character, and, also, one which contains iodine. A particular shell which is best adapted for this use is abalone shell which appears to contain a desirable 70 quantity of iodine as having as its major characteristics, the properties of ground bone as distinguished from the calcium carbonate characteristics of most of the sea shells. The abalone shell has also the property of constituting a de- 75

oxidizer for the materials from which the alloy is formed. Also, this shell has a relatively high vaporization point, assisting the ground glass and borax in forming a coating which floats 5 upon the top of the molten mass and prevents oxidation of the materials within the mass. I also prefer to employ in the flux a small quantity of sodium cyanide; also a small quantity of powdered charcoal, and I may also employ a small 10 quantity of boric acid or potassium chloride.

I prefer to compound the flux in a dry condition and preferably mix the powdered ferro chromium with the flux, thus introducing the chromium into the initial charge at the same 15 time as the flux.

A flux which I find is particularly adapted in the production of a desirable alloy in the quantities hereinbefore set forth includes approximately 4 oz. of boric acid, 3 oz. sodium cyanide, 20 1 lb. of ground glass,  $\frac{1}{2}$  lb. of ground abalone shell,  $\frac{1}{4}$  lb. of powdered charcoal, and 1 lb. of borax, this quantity of each of the ingredients forming a sufficient flux to work successfully with the hereinbefore stated amounts of metal 25 employed in forming the alloy.

It will, therefore, be observed that I have provided an alloy which contains a high percentage of zinc, alloyed with nickel and chromium, which have a much higher melting point than the zinc. 30 This high percentage of zinc is possible only by following the procedure of introducing the zinc directly into and below the surface of the molten nickel-copper mixture, in small quantities, and at a time at which a relatively high melting point flux is employed covering the top of the mixture, since otherwise a considerable loss of zinc would occur due to its vaporization and oxi- 35

dation. Moreover, this introduction of the copper and zinc into the mixture in small quantities enables the large quantity of zinc and copper to be put into the alloy without chilling the molten nickel and causing it to amalgamate, 5 ruining the entire mixture. While I find it simple to introduce the zinc and copper in solid form and permit them to melt in the crucible, either or both of these ingredients may be previously melted and introduced below the surface 10 of the mix and flux in any manner known to those skilled in the art, provided that the rate of introduction is kept low enough to avoid precipitation of the nickel and/or chromium.

While I have shown and described the preferred embodiment of my invention, it is to be understood that I do not wish to be limited to any of the details of construction shown herein, except as defined in the appended claims.

I claim:

1. The method of forming an alloy consisting substantially of copper, nickel, and at least 30% by weight of zinc which consists in forming a preliminary alloy of the nickel and the copper and then introducing the zinc into the molten 25 mass in small charges by immersing each charge below the surface of the mass and holding the same immersed until melted.

2. The method of forming an alloy containing copper, nickel, and at least 30% by weight of 30 zinc, which consists in melting the nickel and copper with a flux containing abalone shell, and then introducing the zinc into the molten mass in small charges by immersing each charge below the surface of the mass and holding the 35 same immersed until melted.

HARLAN J. McFADGEN, SR.